

July 19, 1949.

R. NEIGER ET AL

2,476,758

## PROCESS FOR PREPARING A BLEACHED KERATIN MEAL

Filed July 8, 1946



Inventors  
Richard Neiger  
and Vaclav Nachazel  
By Ernest Holcombe  
of Blass Attorneys

## UNITED STATES PATENT OFFICE

2,476,758

PROCESS FOR PREPARING A BLEACHED  
KERATIN MEAL

Richard Neiger, Maryport, England, and Vaclav Nachazel, Tzlove, near Podmokly, Czechoslovakia, assignors to Messrs. Hornflowa Limited, Maryport, England, a British company

Application July 8, 1946, Serial No. 681,799½  
In Great Britain April 23, 1945

Section 1, Public Law 690, August 8, 1946  
Patent expires April 23, 1965

5 Claims. (Cl. 260—123.7)

1

This invention relates to the process for preparing a bleached keratin meal in a form suitable for use in making moulded articles such as buttons, buckles, electrical insulators and fittings. Keratin is generally derived from ground horns and hoofs of animals but the ground product requires purification before it can be used for making high class moulded articles. When required for making translucent mouldings the keratin must be bleached in order that it may be light in shade or coloured to a variety of delicate shades, and it is generally mixed with artificial resins to give mouldings presenting all the desired characteristics. A bleaching process for keratin is known in which it is first treated with an oxidising agent, washed and then treated with a mild reducing agent such as a dilute solution of sodium hyposulphite. By the process forming the subject of the present invention no bleaching by oxidation is found to be necessary.

It is the primary object of the present invention to purify the keratin first by a selective grinding process in which a large proportion of the impurities can be eliminated. A further object is to provide a simple bleaching process for the selectively ground product, involving only a reducing treatment.

The selective grinding process according to the invention consists in crushing the raw material such as hoofs, and then subjecting the product to a selective grinding and sifting process in which the impurities are largely removed with the particles which pass through the finer meshes of the sieves, while the coarser particles of keratin of a higher degree of purity are separated and subjected to a further stage of grinding.

The bleaching process according to the invention consists in steeping the selected keratin product of substantial purity in dilute ammonia for some hours, separating it from the alkaline solution, acidulating it and bleaching with the aid of a reducing agent.

It has been found that a selective grinding and sifting process which removes a large proportion of the impurities, followed by a simple reducing treatment in which the material is first acted upon by dilute ammonia solution, then neutralised and treated with a reducing agent such as sodium formaldehyde sulphoxyllic acid, with or without sodium hyposulphite in acid medium, enables products to be obtained which give excellent translucent or transparent mouldings with the usual artificial resins. These products lend themselves to colouring or the formation of

2

patterns by spraying through stencils, sifting through stencils, and so forth, or of course opaque mouldings can also be made from them by the addition of pigmenting materials if desired.

It has been found that the raw material, e. g. hoofs, contains a certain variable percentage of impurities both organic and inorganic, which, if not removed from the ground material, contaminate it, and are also very difficult to bleach by any known process. The impurities, even after the bleaching, can be found as dark specks throughout the material, and they impair the uniformity of the moulding as well as the colour. They are also objectionable because they may have an adverse effect on the physical qualities of the mouldings. These impurities may be present in the form of dirt adhering to or embedded in the surface of the hoofs, or as incrustations. The former are very difficult to remove by washing, the latter, of course, cannot be removed by washing at all. In order to remove these impurities the following methods have been developed:

25 After being washed the hoofs are dried in preferably vertical drying shafts for approximately 24 to 36 hours at temperatures below the boiling point of water, up to about 80° or 90° C., and then allowed to cool down to room temperature. By this process most of the free water is removed and the subsequent crushing requires substantially less time than without the previous drying. At the same time the dirt and foreign matter are loosened, part peels off and is separated from the hoofs when passing over sieves at the bottom of the shaft through which the finer foreign matter falls. This mechanical purification may be improved by drawing off air through the drying shafts. The hoofs are first crushed and then, instead of grinding the crushed hoofs in a single grinder in one operation until the desired fineness is reached, the grinding is effected in a series of two or more grinders, each with its own self-contained receivers, elevators, and sieve compartments giving what may be termed a selective grinding process.

The crushing is preferably effected in a hammer mill which breaks up or granulates the hoofs, and the grinding is effected preferably in high speed impact grinders or pulverisers such as pin mills so that the breaking effect in each can be controlled by varying the speed of rotation. The selective grinding process is based on the following theory:

The crushing of the hoofs is facilitated by the presence of encrusted or embedded impurities, which constitute points of weakness in the hoof structure so that impact fracture occurs readily at those points where foreign matter is present. The liberated impurities then pulverise much more quickly to a finer powder than the hoof fragments. The material is then passed over a number of sieves of different mesh, and the finer particles containing most of the impurities and dirt fall through the sieves and are so separated from the coarse material which is then conveyed to the next grinder and the whole process is repeated. It is advisable to grind the hoofs firstly in one or more grinders with a speed of 2000 to 3000 R. P. M. and then in one or more grinders at a higher speed, say 4000 to 6000 R. P. M. The ground material which falls from each of the machines is passed through a separate set of elevators and sieves enabling the various grades to be differentiated both with regard to their mesh size and purity. It is very important to start the grinding at lower speed because the pulverizing action is then gradually increased and favours the selective grinding and separation. The further the process advances the cleaner do the separated materials become.

A suitable lay-out of plant for this purpose is indicated in the accompanying diagram which shows a flow sheet of the plant. The raw material such as hoofs is fed through a preliminary washer *a* to driers *b* through which hot air from a fan *c* is passed. The dried material is raised by an elevator *d* and delivered to a magnetic separator *m*<sup>1</sup> and a hammer mill or crusher *e*. The product from the mill *e* is raised by an elevator *f* and delivered to rotary sieves *g*<sup>1</sup>, *g*<sup>2</sup>, of different degrees of fineness, the fine through products which contain a good deal of foreign matter being collected in sacks *s*<sup>1</sup>, *s*<sup>2</sup>, while the overs are carried by elevator *i* and delivered to bins *k*<sup>1</sup>. A fan *p*<sup>1</sup> extracts dust-laden air from the input end of elevator *f* and the rotary sieves *g*<sup>1</sup>, *g*<sup>2</sup>, the dust being collected in dust collector *o*<sup>1</sup> which delivers it to a sack *h*<sup>1</sup>. From bins *k*<sup>1</sup> the material passes through another magnetic separator *m*<sup>2</sup> to an impact pulveriser *l*<sup>1</sup> which may run at say 3000 R. P. M. Part of the output from pulveriser *l*<sup>1</sup> goes to a cyclone-type separator *n*<sup>1</sup> from which air is extracted through a dust collector *o*<sup>2</sup> by a fan *p*<sup>2</sup>, the dust being collected in sack *h*<sup>2</sup>. Another part of the output goes to one of a series of elevators *q* delivering the product to one of the plansifters *r*<sup>1</sup> to *r*<sup>6</sup>, these being sifting machines having multiple sieve units which are horizontally agitated.

Additional grinding bins *k*<sup>2</sup> and *k*<sup>3</sup> are provided which receive coarser material fed back as overs from some of the plansifters *r*<sup>1</sup> to *r*<sup>6</sup> by certain of the elevators *q*. The output from the bins *k*<sup>2</sup> and *k*<sup>3</sup> is delivered past magnetic separators *m*<sup>3</sup> and *m*<sup>5</sup> respectively to impact pulverisers *l*<sup>2</sup> and *l*<sup>4</sup> running at say 4000 to 6000 R. P. M. and connected to cyclone-type separators *n*<sup>2</sup> and *n*<sup>4</sup>. The major part of the output of pulverisers *l*<sup>2</sup> and *l*<sup>4</sup> goes to the elevators *q* and the plansifters. An intermediate magnetic separator *m*<sup>4</sup>, pulveriser *l*<sup>3</sup> and cyclone-type separator *n*<sup>3</sup> operate upon coarse overs fed back from some of the plansifters *r*<sup>1</sup> to *r*<sup>6</sup>, and return part of the pulverised product to the plansifters again. The pulveriser *l*<sup>3</sup> may run at say 6000 R. P. M. The dust-laden air from separators *n*<sup>1</sup> and *n*<sup>2</sup> goes to dust collector *o*<sup>2</sup> and fan *p*<sup>2</sup>, while dust-laden air from separators *n*<sup>3</sup> and *n*<sup>4</sup> goes to dust collector *o*<sup>3</sup> and

fan *p*<sup>3</sup>. The dust from collector *o*<sup>2</sup> is received in sack *h*<sup>2</sup>, and the dust from collector *o*<sup>3</sup> goes to sack *h*<sup>3</sup>. The graded products from the plansifters *r*<sup>1</sup> to *r*<sup>6</sup> are collected in sacks *s*<sup>3</sup> to *s*<sup>10</sup>. This flow sheet is to be regarded only as one example of a suitable plant.

The products delivered from the various plansifter compartments into sacks *s*<sup>3</sup> to *s*<sup>8</sup> are of different grades and purity depending upon the steps of grinding and sieving which they have passed through. The purest types are well adapted for bleaching, compounding with artificial resins and moulding to give products of a high translucency, suited for colouring, and for further treatment such as surface spraying or sifting through stencils to produce articles resembling natural horn or other materials. The less pure products, as well as those received in sacks *h*<sup>1</sup>, *h*<sup>2</sup>, *h*<sup>3</sup> and *s*<sup>1</sup>, *s*<sup>2</sup> can be mixed with artificial resins and colouring matter to produce good quality opaque articles but are not pure enough to justify refining and bleaching.

It has been proved analytically that the ash content, i. e. the inorganic material in the product received in the sacks *s*<sup>3</sup> to *s*<sup>10</sup> decreases from about 2.5% down to 0.2% in proportion as the grades of the material improve in purity in the course of the selective grinding and sieving process. The material so produced is cleaner and more uniform than the products obtained by the usual grinding methods, and represents an ideal starting material for the further refining treatment. When mixed with an artificial resin and moulded under heat and pressure this material results in a moulding of yellowish colour and milky-opaque appearance. In order to obtain a material giving a moulding of lighter colour and greater translucency, this product requires further treatment, consisting of refining and bleaching. This treatment is preferably effected in the following manner:

Firstly, the material is treated for 16 to 24 hours with an ammoniacal solution of say 0.5% strength. This treatment results in making the product lighter in colour as well as causing a loosening and slight swelling of the keratin substance without however chemically attacking the substance. The subsequent bleaching treatment with a reducing agent, or a combination of agents, has a far better effect than without a preceding ammonia (alkali) treatment.

It is undesirable to employ sodium- or potassium-hydroxide as an alkaline agent, as these chemicals—even in dilute solutions—tend to cause splitting of the protein substance, especially of the cystin. Cystin, which is contained in hoofs up to 15% is easily split up by alkali (caustic) evolving hydrogen-sulphide. When neutralized with acid, colloidal sulphur is formed. The protein is partly destroyed down to the structure of animal glue. This results in a considerable darkening of the moulding caused by oxidation and other reactions catalysed by the heat of the moulding process. We have ascertained that the pretreatment of the hoof substance with dilute (*n*/10) ammonia solutions results in the required loosening of the particles, without the above mentioned disadvantages of NaOH and KOH. Even 4*n* solutions of ammonia do not cause visible destruction of the keratin, whereas, NaOH or KOH would destroy the keratin irreversibly. If the material pretreated in this way is mixed with a resin and pressed under heat, the moulding is of greater translucency and lighter colour than the untreated material. The mould-

ing is also more resistant to water than one obtained from material pretreated with caustic alkalis. A simple reducing treatment following the pretreatment with ammonia completes the preparation of the purified keratin product for use in moulding high class translucent products.

The following are examples of the bleaching treatment:

*Example 1*

|              |                 |      |
|--------------|-----------------|------|
| Hoofmeal     | parts by weight | 550  |
| 0.88 ammonia | parts           | 10   |
| Water        | do              | 1800 |

are agitated for 16 to 24 hours and the water subsequently removed by centrifuging. The material can be washed if required, before placing in 1500 parts of water. The water, which is slightly alkaline to litmus, is neutralised with iron-free hydrochloric acid, and 15 to 20 parts of sodium formaldehyde sulphoxyllic acid are added under constant stirring. The pH value of the solution is then lowered to approximately 4.5 to 5.5 by the addition of acid. By the acidification of the solution the reducing power of the agent is accelerated, and certain impurities are dissolved in the acid medium. It is necessary to adjust the pH value which, at the beginning of the process, has a tendency to rise. The material is then centrifuged, washed with water until the pH value of the washing water remains slightly below 7. The material is finally dried at 45-50° C.

*Example 2*

As in Example 1, with the exception that the bleaching medium is a solution containing 5 parts of sodium hypo-sulphite ( $Na_2S_2O_4$ ) and 10 parts of sodium formaldehyde sulphoxyllic acid. The process is first carried out in alkaline medium, when the hypo-sulphite will start the bleaching, and after the end of this reaction (in which the sodium formaldehyde sulphoxyllic acid plays very little part) the pH value is adjusted to 4.5-5.5 when the reductive power of the latter is brought into action.

*Example 3*

25 parts of hoofmeal in 125 parts of *n*/10 ammonia are maintained at room temperature for 6 hours, with constant stirring. After neutralising and washing, the water is removed and the material put into 90 parts of water at approximately 90 degrees C. in which 0.7 to 1.5 parts of sodium formaldehyde sulphoxyllic acid are dissolved. The temperature is kept up to 70° to 80° C. for 2 to 6 hours. Steaming of the material must be prevented. The material is then centrifuged, washed with water and dried at 45° C.

*Example 4*

As in Example 3, with the exception that the pH value of the bleaching solution is brought down to from 5 to 3 as may be found necessary. It has to be borne in mind that we are dealing with an organic material which varies with the origin of the cattle, and consequently the methods employed have to be varied within certain limits.

All the materials obtained by the methods described in the examples when moulded under heat and pressure show a great improvement in colour and translucency. They can be moulded into many articles, of limited size, as for example small electrical insulators or fittings, buttons and slides. The mouldings have to be hardened in formaldehyde solutions but their resistance to water if moulded without additions of resin, is rather poor.

When incorporated into amino-formaldehyde resins, as for instance urea- or melamine formaldehyde condensation products, moulding powders are obtained which can be moulded at 145° to 160° C., and a pressure of 1 to 1½ tons per square inch. The resulting mouldings are of great clarity without having lost their hornlike appearance, are highly resistant to water, and combine the hard brilliancy of the finish of a synthetic resin with the soft sheen of the natural horn. The mouldings show all the characteristics of the amino-aldehyde resins and can be machined and turned to any required shape. The perfect uniformity of the material makes it possible to obtain the most delicate shades in translucent, semi-transparent and opaque varieties by the usual dyeing methods. The moulding powder has a good flow and cures satisfactorily.

When mixed with phenol-formaldehyde resin the moulding powder can be dyed to a greater variety of shades than the usual wood or cellulose-filled moulding compounds.

Although hoofs have been referred to as the preferred raw material for the ground keratin, horns and other natural materials rich in keratin can be used, but the best quality products are generally made from hoofs in the manner hereinbefore described.

We claim:

- 30 1. A process of preparing keratin meal for use in moulding compositions, consisting in crushing natural animal products of the class consisting of horns and hoofs composed mainly of keratin, and subjecting the crushed product to a plurality of stages of grinding increasing in intensity from one stage to another, and to intermediate sieving, wherein loosened foreign matter is eliminated, the overs from the last stage of sieving comprising keratin meal in a relatively high degree of purity, steeping the keratin meal in dilute ammonia for a period of several hours duration, separating the alkaline solution from the keratin meal, placing the separated product in water, neutralizing it with a weak solution of acid, and stirring into the liquid a reducing agent having bleaching properties containing a substance selected from the group consisting of sodium formaldehyde sulphoxyllic acid and sodium hyposulphite, separating the product from the liquid, washing and drying it.
- 40 2. A process of preparing keratin meal as claimed in claim 1 wherein the reducing agent comprises sodium formaldehyde sulphoxyllic acid.
- 50 3. A process of preparing keratin meal as claimed in claim 1 wherein the reducing agent comprises sodium formaldehyde sulphoxyllic acid and sodium hyposulphite.
- 60 4. A process of preparing keratin meal for use in moulding compositions, consisting of crushing natural animal products of the class consisting of horns and hoofs composed mainly of keratin, and subjecting the crushed product to a plurality of stages of grinding increasing in intensity from one stage to another, and to intermediate sieving, wherein loosened foreign matter is eliminated, the overs from the last stage of sieving comprising keratin meal in a relatively high degree of purity, steeping the keratin meal in dilute ammonia for a period of several hours, centrifuging to separate out the alkaline liquid, adding water to the product, neutralising with iron-free hydrochloric acid, adding a reducing agent having bleaching properties containing a substance selected from the group consisting of sodium formaldehyde sulphoxyllic acid and sodium
- 70
- 75

hyposulphite, adding more acid to lower the pH value of the liquid to 5.5 or less, centrifuging the product, washing and drying the product.

5. A process of preparing keratin meal for use in moulding compositions, consisting in crushing natural animal products of the class consisting of horns and hoofs composed mainly of keratin, and subjecting the crushed product to a plurality of stages of grinding increasing in intensity from one stage to another, and to intermediate sieving, wherein loosened foreign matter is eliminated, the overs from the last stage of sieving comprising keratin meal in a relatively high degree of purity, steeping the keratin meal in dilute ammonia for a period of several hours duration, adding a reducing agent having bleaching properties comprising a mixture of sodium hyposulphite and sodium formaldehyde sulphonylic acid, and subsequently adding acid to reduce the pH value of the liquid below 5.5, separating the product from the liquid, washing and drying it.

RICHARD NEIGER.  
VACLAV NACHAZEL.

## REFERENCES CITED

The following references are of record in the file of this patent:

## UNITED STATES PATENTS

| Number       | Name               | Date           |
|--------------|--------------------|----------------|
| 687,219      | Gaff               | Nov. 26, 1901  |
| 867,167      | Stiegelmann et al. | Sept. 24, 1907 |
| 1,594,633    | Schar              | Aug. 3, 1926   |
| 10 2,072,665 | Campbell et al.    | Mar. 2, 1937   |

## FOREIGN PATENTS

| Number | Country       | Date          |
|--------|---------------|---------------|
| 15 423 | Great Britain | Apr. 11, 1856 |

## OTHER REFERENCES

Lehmann: Melliand Textil Berichte, vol. 24, pp. 1 to 5 (Jan. 1943).